

# UNITED STATES PATENT OFFICE.

HUGH S. COOPER, OF CLEVELAND, OHIO, ASSIGNOR, BY MESNE ASSIGNMENTS, TO  
ZIRCON TOOL & ALLOY CORPORATION, A CORPORATION OF NEW YORK.

## ALLOY.

1,350,359.

Specification of Letters Patent. Patented Aug. 24, 1920.

No Drawing.

Application filed August 22, 1918. Serial No. 250,929.

To all whom it may concern:

Be it known that I, HUGH S. COOPER, a citizen of the United States, residing at Cleveland, in the county of Cuyahoga and State of Ohio, have invented certain new and useful Improvements in Alloys, of which the following is a specification.

This invention relates to a high-speed cutting tool alloy comprising nickel, zirconium, aluminum and silicon, in the proportions substantially as hereinafter described and more particularly pointed out in the claims.

In my Letters Patent of the United States No. 1,221,769, dated April 3, 1917, filed Oct. 15, 1916, I disclose the use of small percentages of zirconium together with a preponderating amount of nickel or cobalt to produce an alloy especially adapted for use in making high-speed cutting tools. In producing said zirconium-nickel alloy, I practised various methods of manufacture, one being the alumino-thermic method, and I have made many different species of nickel-zirconium alloys, using nickel oxide, zirconium silicate, powdered aluminum, and an ignition powder, with and without a metal of the chromium group. In analyzing such alloys made from oxides obtainable on the market and casting the product in carbon 25 molds, a small percentage of carbon and iron 30 will usually appear.

In making such alloys I found that a preponderating amount of nickel, together with silicon and aluminum, and one-half to fifteen 35 per cent. of zirconium would yield a very hard and tough cutting-tool metal, and that a relatively small amount of zirconium was required where the aluminum and silicon together substantially exceeded the amount of 40 zirconium used. Thus, in my application for Letters Patent for an alloy, filed Feb. 23, 1918, Ser. No. 218,791, I show that an alloy of approximately equal parts of silicon and aluminum, with the balance nickel, will be 45 greatly improved for cutting purposes by the addition of one-half to about fifteen per cent. zirconium. I also found that an increased hardness was obtained with higher percentages of aluminum and lower percentages of silicon, and that the alloy may contain from one to ten per cent. silicon, one to 50 twelve per cent. aluminum, and less than two per cent. of zirconium. Moreover, small

amounts of one or more of the metals of the chromium group, for example, tungsten may 55 also be used with beneficial results.

One species of a composition which I have made and tested and found to give efficient cutting service, contained 5.9% or approximately six per cent. of silicon, 1.9% or approximately two per cent. of aluminum, 60 4.8% of zirconium, 3.8% of tungsten, 6.8% of iron, .29% of carbon, and 76.2% of nickel.

Another alloy which also gave excellent cutting results, and in which the amount of 65 zirconium used was less than two per cent., contained a preponderating amount of nickel, aluminum 2.9%, silicon 6.8%, zirconium 1.9%, tungsten 7.3% and small amounts of iron and carbon not exceeding six per 70 cent.

Still another alloy made and tested by me, which gave satisfactory service as a cutting tool alloy, contained 1.6% of zirconium, 5.4% silicon, 8% aluminum, with the balance nickel and showing a small per cent. 75 of iron where baddeleyite was used.

It will be noted from the foregoing that a serviceable alloy for high speed cutting tools may contain a preponderating amount 80 of nickel, one-half to two per cent. of zirconium, and aluminum and silicon together at least double the amount of zirconium. The aluminum and silicon may each constitute from two to eight per cent. of the alloy, 85 but where a small amount of zirconium is used, not exceeding two per cent., the aluminum should not exceed ten per cent. and the silicon should not exceed six per cent.

The most desirable alloys contain aluminum in excess of silicon. However, where the zirconium exceeds two per cent. and the silicon is approximately six per cent., the amount of aluminum must be reduced below ten per cent. and may be as low as two per cent. This is illustrated in the first species of alloy given above to show that the use of a larger proportion of zirconium than two per cent. is not prohibitive.

In producing the alloy, either pure oxide 100 of zirconium, the native silicate, commonly called zircon, or the native oxide known as baddeleyite, may be used. The last two minerals can be used without purification and are mixed in the proper proportions with 105 the oxide of nickel and powdered aluminum.

The natural silicate of zirconium contains from sixty-one per cent. upward of the oxid with the balance silica, and in the process of reduction, using aluminum as a reducing agent, the product will contain zirconium, silicon and aluminum in various proportions dependent upon the proportions of the mixture. Where the native zirconium minerals are used a small percentage of iron is usually present in the alloy, but this small content has no appreciable effect upon the cutting qualities or efficiency of the alloy.

By a preponderating amount of nickel I mean from seventy to ninety per cent., and in making the alloy by reduction with powdered aluminum if it is found that the alloy is too hard for the amount of nickel used, more nickel is added after transferring the molten alloy to a standardizing furnace, and powdered tungsten may then also be introduced into the alloy, if desired.

What I claim is:

1. An alloy for high speed cutting tools containing a preponderating amount of nickel, zirconium one-half to two per cent., and an amount of aluminum and silicon at least double the amount of zirconium.
2. An alloy for high speed cutting tools containing a preponderating amount of nickel, zirconium one-half to two per cent., and aluminum and silicon each of the last two metals constituting from 2 to 8 per cent. of the alloy.
3. An alloy for high speed cutting tools containing a preponderating amount of nickel, zirconium not less than one-half per cent., and from 8 to 16 per cent. of aluminum and silicon.

Signed at Cleveland, in the county of Cuyahoga, and State of Ohio, this 10 day of August, 1918.

HUGH S. COOPER.